

March 3, 1964

J. F. BYRNE

3,123,474

PHOTOGRAPHIC COMPOSITION

Filed Oct. 21, 1960



*Fig. 1*



*Fig. 2*

INVENTOR.

JOHN F. BYRNE

BY *Frederick F. Lange*

ATTORNEY

# United States Patent Office

3,123,474  
Patented Mar. 3, 1964

1

3,123,474

## PHOTOGRAPHIC COMPOSITION

John F. Byrne, Columbus, Ohio, assignor, by mesne assignments, to Minneapolis-Honeywell Regulator Company, Minneapolis, Minn., a corporation of Delaware

Filed Oct. 21, 1960, Ser. No. 64,192

10 Claims. (Cl. 96—108)

The present application is a continuation-in-part of my copending application Serial No. 737,831, filed May 26, 1958, now abandoned.

The present invention relates broadly to photographic sensitive films and more particularly to photographic films of the "print-out" type. The term "print-out" refers to that type of photosensitive substance upon which a visible image is obtained after an initial exposure to light or electromagnetic radiation has been utilized to form a latent image, the visible image being obtained initially or simply by an additional exposure to such radiation. This additional exposure is known as "latensification" and is general in its application, including exposing the area upon which the initial image was formed as well as the surrounding background area to an added amount of radiation. Print-out emulsions are distinguished from development emulsions which require a development treatment such as a chemical development after initial exposure to produce a visible image, inasmuch as this image is produced by an additional exposure in print-out emulsions. The specific "print-out" papers coated with a film, comprising a dispersion or emulsion of the compositions of the present invention are particularly sensitive to a high intensity beam of light or other electromagnetic energy of either visible or invisible wavelength radiated across a portion of the area of the film. While the material of the present invention is particularly sensitive to such exposure, the background or non-exposed area is sufficiently stable to render a highly contrasting image upon subsequent "latensification".

According to the present invention, a photosensitive silver halide is used as the basic sensitive ingredient of the composition, and a quantity of lead halide is added to the silver halide in order to improve the photo response thereof. The lead halide sensitizes the silver halide particularly to brief exposures, in the range of microseconds, from a high intensity source, but causes very little sensitization of the composition to relatively lower intensity radiation. A high degree of sensitivity to the trace coupled with a highly stable background produces a maximum contrast between the image and the background when applied to recording operations. The present invention provides this desirable combination of high image sensitivity and high degree of background stability.

The intensity of the radiation source utilized in latensification is not as critical with the sensitive mixtures of the present invention as it is with available compositions of the prior art. In other words, the accumulated quantity or intensity of illumination or radiation to which the sensitized paper is exposed during latensification is not particularly critical. The latensification rate obtainable by an intense exposure to ordinary fluorescent lamp lighting conditions has been found to be satisfactory for the silver halide compositions of the present invention, while this intensity of light is generally too great for emulsions produced prior to the present invention.

The term "halide" as used throughout the specification is intended to encompass bromides and iodides, fluorides and chlorides being specifically excluded. Accordingly, the silver halide consists mainly of or entirely of silver bromide although the use of a mixture of predominantly silver bromide with a minor quantity of silver iodide has proved particularly useful.

2

In the early development of photography, "print-out" papers were relatively widely used for ordinary photographic purposes. With the advent of improved development emulsions, "print-out" emulsions fell into a more and more limited use and this situation continued until only recently when it was recognized that they possessed desirable properties for high speed recording such as oscillographic recording and the like. As an example, such a recording system is disclosed in the co-pending application of Mahoney et al., Serial No. 638,729, filed February 7, 1957, and entitled "Recording Apparatus." Unfortunately, the sensitive papers and sensitive coating substances of the prior art are not entirely satisfactory for this recording purpose for a number of reasons. For example, it is generally true that the prior art papers which exhibit high sensitivity to an exposure of short duration to a high intensity beam tend to exhibit a correspondingly low degree of background stability. The printing out or latensification procedure for these sensitive papers is highly critical and accordingly is exceedingly difficult if not impossible to carry out. The latent image may be entirely lost during the subsequent latensification operation due to the fact that the background "comes up" or "points-out" too rapidly. In other cases a phenomenon known as "reversal" may occur, this being a darkening of the background which proceeds at a more rapid rate than darkening of the image or trace. In these situations, the trace may be temporarily or permanently lost. On the other hand, papers which exhibit a high degree of background stability tend to exhibit a correspondingly low degree of sensitivity to the recording beam and accordingly the maximum writing speed (minimum exposure time) is far below that desired for use with modern recording instruments.

Hence, when it is attempted to produce a latent image upon a low sensitivity paper at an excessive rate for the paper, the image, if formed at all, will become lost against the background upon print-out.

In addition to these problems, it is also critical that the sensitive paper exhibit a certain degree of permanence in order that any record prepared thereon will have a sufficiently long and usable lifetime without losing its contrast. It is also desirable to have a sensitive paper which responds substantially uniformly to applied radiation without regard to varying intensities and different writing speeds and yet which exhibits a substantially uniform degree of contrast against the background upon latensification. According to the present invention, the sensitive films possess a sensitivity capable of writing in a wide range of speeds, including very slow speeds as well as speeds ranging up to more than 50,000 lineal inches per second. In spite of the varying requirements relative to different writing speeds, a uniform, relatively permanent, and highly contrasting image is produced upon latensification. Latensification may be accomplished through exposure to radiation within the sensitive range for the paper for a very short period of time. For example, several seconds or less under an ordinary fluorescent lamp is sufficient to latensify or print-out the images or traces made on paper prepared in accordance with the present invention.

Accordingly, it is an object of the present invention to provide improved "print-out" sensitive coating compositions which possess both a high degree of sensitivity to a trace recording along a portion thereof together with a high degree of background stability upon general latensification.

It is a further object of the present invention to provide "print-out" sensitive coating compositions which produce an image or trace which has a substantially uniform degree of contrast to the background, this contrast being relatively independent of the time the sensitive material

has been exposed to a relatively intense and uniform light source.

It is yet another object of this present invention to provide a "print-out" emulsion which produces a latent invisible image after an initial exposure time in the range of microseconds, and which will "print-out" the latent image upon an exposure of general application of short duration.

It is still a further object of the present invention to provide a photosensitive "print-out" sensitive coating composition which is exceedingly fast in its photographic response, which is substantially stable over a long period of time, and which may be retained for an indefinite period of time so long as it is not exposed generally to light or other electromagnetic radiation for extended periods.

Other and further objects will become apparent to those skilled in the art upon the study of the following specification, appended claims and accompanying drawings wherein,

FIGURE 1 is a schematic illustration of a preferred process for preparation of sensitive dispersions in accordance with the present invention; and

FIGURE 2 is a cross sectional view showing the sensitive material as a coating on a support member.

The exact theory of operation of the compositions of the present invention is not entirely understood. In silver halides generally, and in particular silver bromide, exposure to light produces elemental silver and free bromine, this phenomenon probably being carried out in accordance with the reversible equation shown below.



Applied to the present case, the free silver indicates the exposed area and a darkening of the area occurs. When the light or other electromagnetic radiation is removed, the reaction in general may tend to reverse and therefore proceed to the left with a consequent loss of indicated exposed area. Silver halide emulsions have long been employed in the photographic art, including silver bromide and silver bromo-iodide as employed in the present invention. The presence of lead halide is believed to prevent reverse reactions from occurring and hence increases stability. The useful halides of lead consist of both lead iodide and lead bromide. Lead iodide has been found to be markedly superior as a doping agent with silver halide to other compounds of lead, although lead bromide has also been found useful in the invention. The sensitivity achieved with lead bromide is essentially the same as that producible with lead iodide, however, both the iodide and bromide are superior by a considerable margin over other lead salts such as chloride, nitrate, acetate, etc. The writing speed of compositions containing other lead salts is lower, and the trace, if formed, tends to fade and in some cases is substantially assimilated into the background.

By way of theoretical explanation for the improvement obtained with lead halide additions as applied to compositions under consideration here, it will be appreciated that precise descriptions of the mechanisms involved are difficult to set forth. It does appear however, that the lead halide functions as an acceptor for the bromine liberated by light energy on the silver bromide. It is believed that this could be by way of an oxidation of lead from a valence of +2 to a valence of +4, by a displacement of the iodide ion by bromine, or even by a combination of these phenomena.

Referring now to the lead halide additions, the relative proportion of lead halide added to the silver halide has been found to be beneficial only if held within certain limits. In cases where less than 0.1% of lead halide by weight has been added to the silver halide sensitive mixtures, a phenomenon known as "reversal" has occurred. In these instances, as previously indicated, the latent

image is either temporarily or permanently lost or rendered without contrast against the background upon latensification. If lead halide is added in excess of about 20% by weight, the emulsion tends to become quenched and is substantially less sensitive. Thus, in the range between 0.1% and 20%, and in particular the range between 1% and 5%, there is found to be an optimum relationship between sensitivity of film and stability of background.

10 The lead halide additive, as noted above, performs substantially as a bromine acceptor, and hence there is no requirement that conventional bromine acceptors such as gelatin or the like be present in the compositions of the invention.

15 It has been found that a small percentage of silver iodide when added to the silver bromide enhances the sensitivity of the emulsions. In this connection, amounts ranging from about 1% to about 10% of the co-precipitated silver iodide have been found useful, and specifically

20 about 5% of silver iodide appears to give optimum results. In this connection, it is believed that the silver iodide being present in the lattice sets up strains in the silver bromide lattice to such an extent that reduction of silver to the free metal is achieved more easily, and this 25 reduction is rendered somewhat more stable in nature. Although the invention is operable using a single halide salt, e.g., AgBr, or with a mechanical mixture of AgBr plus AgI, the co-precipitated silver bromo-iodide is preferred.

30 The compositions of the present invention may be further sensitized if desired, by adding from .01 to .2% (by weight based on total solids) of an organic sensitizer such as thiourea which is the preferred sensitizer for this composition. Thiocarbamide, thiosemicarbazide, para-methylamino phenol sulphate and mercapto succinic acid are useful and may be employed if desired.

Various inert carriers or binders, and particularly organic colloid carriers, may be employed in order to facilitate application and adhesion of the sensitive composition

40 to paper in dispersion or emulsion from either aqueous compatible or aqueous incompatible carriers may be employed. In an aqueous system, pre-gelatinized dextrin gelatin, starch, dextrin, thickening agents such as seaweed extracts or polyvinyl alcohol are suitable. In the 45 nonwater-soluble systems, silicones may be employed. The carriers do not in any way affect the photographic properties of the compositions, but are merely used to adhere the composition to the base material.

Among the various base papers or supports, one may 50 employ almost any sort of cellulose paper so long as it is free from wood chips or the like. Conventional photographic base papers may be conveniently utilized.

Heat treating the coated paper when carriers other than gelatin have been used has been found advantageous in increasing top writing speeds and retarding the rate of

55 background rise. In this connection, heating to a temperature of about 400° F. for a period of from 10 to 30 seconds produces beneficial results. Specifically a temperature of about 400° F. for a period of about 20 seconds has been considered the optimum for compositions 60 prepared in accordance with the present invention.

For exposure and latensification, the maximum sensitivity of the paper is found to be below about 5000 Angstroms, and mainly below about 4400 Angstroms. Various 65 commercially available high intensity light sources may be conveniently employed for producing the trace image, such as for example the Osram lamp manufactured by Osram, Munich, Germany, as hereinafter identified in Example 1. By the term "high intensity radiation" reference is made to electromagnetic radiations having an intensity of about 10<sup>8</sup> ergs/sec./cm.<sup>2</sup> or greater. In order to obtain a useful trace, this is preferably applied to the paper for a period of about 10<sup>-6</sup> seconds or greater. Although lower intensity sources may be satisfactorily utilized, these sources may require substantially

higher total energies inasmuch as the material exhibits a low intensity reciprocity failure.

While the sensitive films are particularly sensitive to radiations of relatively high intensity, they are also suitable for use at lower intensities, with a corresponding drop in writing speed. For latensification, a less intense source of light available generally across the extent of the paper is desired. Ordinary fluorescent lighting at close range is useful both in its intensity and its output wave lengths characteristic for latensification operation. For example, latensification may be carried out under the influence of illumination of the order of 75 foot-candles of "cool-white" fluorescent light.

In order to more particularly set out the features of the present invention, specific examples of preparation are presented hereinbelow:

#### EXAMPLE 1

In the preferred embodiment of the present invention, the following preparation is recommended.

##### Preparation of Silver Nitrate

|                                                         | Amount             |
|---------------------------------------------------------|--------------------|
| AgNO <sub>3</sub>                                       | 187 gr. (1.1 mol). |
| H <sub>2</sub> O (distilled)                            | 500 cc.            |
| NH <sub>3</sub> (28-30% aqueous solution, sp. gr. 0.90) | 200 cc.            |

The silver nitrate was weighed and dissolved in the prescribed amount of distilled water. This solution was heated to about 60 to 65° C. Then the ammonia solution was added with stirring until the solution cleared as the precipitate of silver oxide formed by the first added portions of the ammonia was redissolved.

##### Potassium Halide Solution

|                              | Amount                |
|------------------------------|-----------------------|
| KI                           | 9.13 gr. (0.055 mol). |
| KBr                          | 137 gr. (1.15 mol).   |
| H <sub>2</sub> O (distilled) | 500 cc.               |

The potassium iodide was weighed carefully in order to insure precise control over the iodide content of the resultant silver halide mixture. The potassium halides were dissolved in the prescribed amount of water contained in two liter beakers which was set in a water bath. The water bath was provided with an inlet through which steam was introduced to heat the bath to about 95° C. The solution of potassium halide was stirred mechanically with the glass-rod stirrer driven by an air turbine.

##### Preparation of Silver Bromoiodide

When the halide solution was hot (85 to 90° C.) the ammoniacal silver nitrate solution was added slowly in a steady stream to the reaction vessel. This was done by pouring the silver solution slowly into a funnel to the outlet of which has been fused a short length (about 4 inches) of capillary tubing. The capillary jet delivered the silver solution at a rate of about 50 cc. per minute, so that the addition of silver was completed in about 15 minutes. The iodide reacts preferentially because of its being less soluble than the silver bromide. In this connection, there may be considerable co-precipitation so that silver iodide is trapped in silver bromide crystals with the result that strained crystals of high sensitivity are formed.

Ammonia and potassium bromide act as solvents for the silver halides formed and promote crystal growth. Thus, in the presence of these solvents, the smaller silver halide crystals may dissolve and be re-deposited on the surfaces of larger crystals by a process known as Ostwald ripening. This process can occur during the slow precipitation step and also during the ripening step which follows the precipitation. The silver halide precipitate was ripened by maintaining the reaction vessel at 85 to 90° C. for a period of about 20 minutes after all of the silver nitrate had been added, the mixture being stirred moderately with a mechanical stirrer during the ripening period.

After the ripening step, the silver halide mixture was filtered by suction on a Buchner funnel and was washed five times with distilled water.

It is not normally necessary to dry the silver halides after filtering and washing. If it is desired to dry the silver halides, this may be done in an oven at 220-230° F. but can also be accomplished by exposure to low humidity air for about 24 hours.

##### Compounding of Print-Out Coating Mixture

In addition to silver bromoiodide, the following ingredients were utilized in preparing a preferred mixture in accordance with the present invention.

Lead iodide—to increase the print-out effect (and to suppress background during latensification).

Thiourea—to sensitize the halide mixture.

Dextrin—to bind the coating to the paper support.

##### Compound:

|                                            | Amount                                          |
|--------------------------------------------|-------------------------------------------------|
| 20 Silver halide (as prepared hereinabove) | 98 gr.                                          |
| Lead iodide                                | 2 gr.                                           |
| 25 Thiourea                                | 0.1 gr. (dissolved in 10 cc. H <sub>2</sub> O). |
| Dextrin (pregelatinized)                   | 4 gr. (dissolved in 40 cc. H <sub>2</sub> O).   |
| H <sub>2</sub> O (distilled)               | 25 cc.                                          |

The ingredients listed above were placed in the eight ounce amber bottle of a ball-mill containing 200 grams of one-half inch porcelain pebbles. The bottle was rotated at about 100 r.p.m. for a period not exceeding about four hours, after which time a homogeneous mixture resulted. The mixture described above had a consistency which was found suitable for making flow-coated papers.

35 After milling it is convenient to mix the material prepared as above with an aqueous solution of a suspending agent to hold the silver halide particles in substantially uniform distribution for applying to paper in a subsequent coating operation. One such suspending agent found to be satisfactory is a sea-weed extract which was used in a one percent solution. It will be appreciated that this suspending agent should not adversely react with the sensitive materials. Sea Kem No. 402 is satisfactory in this respect. After mixing into the suspending agent, the compositions are ready for application to the paper. In this connection various application techniques may be employed, such as transfer roller coating, dip coating using an air-knife to wipe off the excess upon emergence from the bath, or by conventional spreading using a doctor knife to control the thickness of the film. Although the thickness of the coatings to be applied to paper or other supports is dependent on the characteristics desired in the end product, it has been found that the composition disclosed above diluted to 600 cc. with 45 water containing 1 percent Sea Kem 402 deposits useful coatings when applied in layers calculated to be in the range of from 2 to 10 mils in thickness. As the thickness of the wet film is difficult to measure, it is somewhat easier to use the weight per unit area of solids deposited 50 as a reference. About 1 gram of solids per square foot of the dried film appears to be satisfactory. The critical features are that the coating be uniform, flexible, and adherent to the base material. After application to the base paper, the coating was dried and was subjected to a 55 temperature of about 400° F. for a period of 20 seconds.

Attention is directed to FIGURE 2 of the drawings wherein there is illustrated a photosensitive paper 10 having a base support 11 and a sensitive coating 12. This coating was prepared as in Example 1 above.

70 The sensitive material prepared in accordance with Example 1 above and shown in FIGURE 2 was yellow in color and upon the desired exposure to light, a uniform medium dark brown image or trace having extremely fine edge definition was formed. Sensitive papers prepared according to this process were capable of writing speeds



precipitate was used at once to make a coating mixture as follows:

300 g. (+ wetness)  $\text{AgBr}-\text{PbBr}_2$  (20:1=mol Ag:mol Pb  
60 cc. of 5% aqueous pregelatinized dextrin solution

This composition was ball milled for 23 hours, and then made into a coating mixture utilizing a small quantity of thiourea in a quantity as indicated hereinabove. A coating prepared from this composition was found to have a sensitivity approximately equal to those of other solutions of the above examples.

Other and further modifications may be employed without departing from the spirit and scope of the present invention. It will be appreciated of course, that the foregoing examples are given for purposes of illustration only and there is accordingly no intention to limit the scope of the present invention to these particular modifications.

I claim:

1. A photosensitive print-out composition comprising a photosensitive substance, said substance consisting essentially of from about 0.1% to 20% by weight lead halide, the balance of said substance being a precipitated washed silver halide, said lead halide selected from the group consisting of lead bromide and lead iodide, said silver halide containing up to 10 mol percent of silver iodide, the balance being silver bromide.

2. A photographic print-out composition comprising a photosensitive substance, said substance consisting essentially of from about 0.1% to 20% by weight lead halide, the balance of said substance being silver bromide, said lead halide selected from the group consisting of lead bromide and lead iodide.

3. A photographic print-out composition comprising an inert carrier having dispersed therein a photosensitive substance, said substance consisting essentially of about 2% by weight lead iodide, the balance of said substance being a precipitated washed silver bromide.

4. A photographic print-out composition comprising an inert organic carrier having dispersed therein a photosensitive substance, said substance consisting essentially of from greater than 0.1% up to about 20% by weight lead iodide, the balance of said substance being a precipitated washed silver halide, said silver halide containing up to about 10 mol percent of silver iodide, the balance being silver bromide.

5. The photographic print-out composition of claim 4 being further characterized in that the photosensitive substance contains greater than about 1% up to about 5% by weight of lead iodide homogeneously dispersed therein.

6. A photographic print-out composition comprising an organic colloid carrier having dispersed therein a photosensitive substance, said photosensitive substance consisting essentially of 2% by weight of lead iodide, the balance of said substance being a washed precipitated silver halide, said silver halide containing up to 5 mol percent silver iodide, the balance being silver bromide.

7. A photographic print-out emulsion sensitive to high intensity radiation of short duration including a film of photosensitive substance dispersed in an organic colloid carrier, said photosensitive substance consisting essentially of from about 1% to about 5% by weight of lead iodide, the balance of said substance being silver halide,

said silver halide containing up to 10 mol percent silver iodide, the balance being silver bromide, said photosensitive substance having added thereto from .01% up to 0.2% by weight thiourea.

5 8. A photographic print-out emulsion sensitive to high intensity radiation of short duration including a film of photosensitive substance dispersed in pregelatinized dextrin, said photosensitive substance consisting essentially of from about 1% to about 5% by weight of lead halide, the balance of said substance being silver halide, said lead halide selected from the group consisting of lead bromide and lead iodide, said silver halide containing up to about 10 mol percent silver iodide, the balance being silver bromide.

10 15 9. A process for the production of photographic print-out emulsions sensitive to high intensity radiation of short duration and including an inert colloid carrier having a photosensitive substance consisting mainly of silver halide and lead halide dispersed therethrough, said process comprising co-precipitating a slurry of silver halide salts wherein from 90 mol percent to 99 mol percent of the silver halides is silver bromide and the balance silver iodide, maintaining said slurry at a temperature of between 85° and 90° C. for a period of about 20 minutes, washing said precipitate, dispersing an amount of lead halide of the class consisting of lead bromide and lead iodide into said silver precipitate in an amount equal to from 0.1% up to about 20% by weight of said lead halide-silver halide mixture, and dispersing said photosensitive substance in an inert colloid carrier.

20 30 35 40 45 10. A process for the production of photographic print-out paper sensitive to high intensity radiation of short duration and including a support element coated with an inert colloid carrier and having a photosensitive substance consisting mainly of silver halide and lead halide dispersed therethrough, said process comprising co-precipitating a slurry of silver halide salts where at least 80 molar percent of the silver halide is silver bromide and the balance silver iodide, washing said precipitate, dispersing an amount ranging between about 0.1% and up to about 20% by weight of lead halide based on the weight of the silver halide-lead halide mixture into said silver halide, said lead halide selected from the group consisting of lead bromide and lead iodide, forming a dispersion of said silver halide and lead halide in an inert colloid carrier, coating a support member with a film of said dispersion, and heating said film to a temperature of about 400° F. for a period between 10 to 30 seconds.

50 References Cited in the file of this patent

UNITED STATES PATENTS

|           |              |               |
|-----------|--------------|---------------|
| 2,816,029 | Jones        | Dec. 10, 1957 |
| 2,843,490 | Jones        | July 15, 1958 |
| 3,039,871 | Scott        | June 19, 1962 |
| 3,047,392 | Scott et al. | July 31, 1962 |

OTHER REFERENCES

- Mueller: Sci. et. Ind. Phot., 24, 494 (1953). (Copy in Sci. Lib. 96-108.)  
German et al.: Journal of Physical Chemistry, 34, pages 1944-1952 (1931). (Copy in Sci. Lib.)